

## UNITED STATES PATENT OFFICE

2,326,690

## COMPOSITION STORAGE BATTERY SEPARATOR AND METHOD OF MAKING THE SAME

Bruno H. Schubert, Weehawken, N. J., assignor to  
National Lead Company, New York, N. Y., a  
corporation of New Jersey

No Drawing. Application October 2, 1941,  
Serial No. 413,300

9 Claims. (Cl. 136—146)

The present application is a continuation-in-part of my copending application, Serial No. 267,-923, filed April 14, 1939, which issued as U. S. Patent No. 2,290,496 on July 21, 1942.

The invention herein described and claimed relates to storage batteries of the lead-acid type, particularly having reference to the use in such types of storage batteries of an improved separator manufactured according to the method herein described. The objects of the invention include, among others, the manufacture of an improved type of storage battery separator as well as the use of such improved separator in storage batteries of the lead-acid type, thereby to impart to the storage battery an improved discharge capacity and a longer life. The novel separators of the present invention are characterized in that they contain as an integral part thereof an added active organic ligneous compound.

By the term "organic ligneous compound" as used in the description of the present invention are meant all of those organic materials of extremely complex chemical nature which are present in all forms of vegetable matter other than the cellulose, fats, waxes, resins, wood acids and salts of wood acids, and said turn also embraces the derivatives of such complex chemical materials, addition and decomposition products thereof. For a better understanding of such complex organic ligneous compounds, reference is made to the book, "Humus" by Selman A. Waksman (The Williams and Wilkins Company, Baltimore, Md.), second edition 1938, page 99.

It is not possible to state what is the true chemical nature of lignin or of organic ligneous materials; chemical science has not yet determined the structure thereof. It is known, however, that when substances of vegetable origin are suitably treated with acidic materials such as calcium acid sulfite, alkalies or some organic solvents, such as dioxane, there are obtained solutions containing among other things some of the ligneous materials originally present in the vegetable substances. Separated from the naturally occurring fats, waxes, resins, wood acids and salts of wood acids also present in the vegetable substance the organic ligneous materials, I have found, possess properties which are conducive to better battery performance when added to separators, and I have designated such ligneous compounds in the description of the present invention and in the appended claims as "active organic ligneous materials." Such a designation will serve to distinguish over those unextracted inactive ligneous compounds which are originally found and which

remain, after treatment, in the structure of the wood. Inasmuch as these organic ligneous compounds are present in all forms of vegetable substances, the particular type of vegetable substance from which the active organic ligneous compound is derived is of no consequence in the practice of the present invention. Wood is a very convenient source for obtaining these active organic ligneous compounds, as are also straw, hemp, jute, corncobs, bagasse, humus, peat moss, etc. The so-called "waste sulfite liquors" obtained from the manufacture of paper or solutions resulting from caustic alkali or inorganic acid processes for treating wood or wood pulp, are a readily available source of organic ligneous compounds, useful in the practice of the invention. On the whole, the sources from which active organic ligneous materials may be derived are well understood by those skilled in the art.

It has been known, prior to our invention, that if lignin and ligneous materials be incorporated into the negative plate of a lead-acid type storage battery, certain desirable effects, in the nature of greater discharge capacity, were imparted to the storage battery. In the manufacture of storage battery separators the most commonly employed material used up to now has been wood. A separator fashioned from wood is treated, for example, with caustic alkali solutions, to remove from the wood the naturally present fats, waxes, resins, wood acids, salts of wood acids and some of the ligneous materials because the art had observed that such compounds as present in the wood in their original states are subject to hydrolysis in the storage battery to the detriment thereof. The so-treated separator, as employed by the prior art, was therefore substantially free of any fats, waxes, resins, wood acids, salts of wood acids, all of which are regarded as detrimental to storage batteries of the lead-acid type.

As noted above, in the treatment of wood separators with caustic soda solution, there is removed in addition to the fats, waxes, resins, wood acids, and the like some of the ligneous material which is uncombined or loosely combined in the wood structure, possibly 2-3% of the total ligneous substance content. A large proportion of this ligneous substance present in the wood is not affected by the caustic soda treatment, probably because it is firmly combined with the cellulose structure of the wood. At any rate, this so-called hemicellulose ligneous organic combination apparently is ineffective in producing improved separators, and I have found it to be necessary to add the so-called active ligneous

material to the treated wood separators in order to impart to a storage battery improved life and low temperature capacity.

Therefore, it should be understood that untreated wood separators do not exhibit the improved properties of my treated separators, and that the ligneous material originally available in the wood is not in the proper active form to produce the desired improvements. Furthermore, it has been found desirable, in the practice of my invention, to effect a uniform distribution of the active ligneous compounds over the surfaces of the separators with sufficient penetration to anchor the products when the organic is set by the acid-fixing treatment.

While pre-fabricated separators have been mentioned above in order that a clearer understanding of the background of the present invention may be had, it is to be understood that the present invention is concerned with composition separators and methods for preparing the same. The treatment of prefabricated separators has been more fully described and claimed in my copending application, Serial No. 267,923, now U. S. Patent No. 2,290,496, dated July 21, 1942, of which as hereinabove mentioned, the present application is a continuation-in-part.

According to the present invention, I have found that if an active organic ligneous compound, either in the form of a dry powder or as a liquid is incorporated as one of the constituents from which a separator is compounded, the resulting so-called composition separator has the unusual property of imparting greater discharge capacity and a longer life to the storage battery.

In the manufacture of composition separators suitable for use as insulating media in storage batteries, any of the well known ingredients suitable for the purpose may be employed, depending upon the particular manufacturer's choice.

Fundamentally, the ingredients will comprise a rubber vehicle, either of the latex type, the gum type or a combination of both. In addition, the ingredients will include suitable vulcanizing agents and accelerators in addition to fillers or porosity agents such as wood pulp, bentonite and the like, and in the case of my improved separators, an active organic ligneous compound in amounts between about 0.01 per cent and about 5.0 per cent of the weight of the separators and preferably between about 0.25 per cent and about 2.0 per cent. In order to illustrate suitable ingredients that may be used in manufacturing composition separators, a specific example is given below. It is to be understood, however, that this example is given for illustrative purposes only and that my invention is not to be limited to the specific ingredients therein recited. The main objective of the present invention resides in the addition of an active organic ligneous compound to the constituents of the separator, thereby to improve battery performance, especially at low temperatures.

#### Example

Composition separators were prepared by thoroughly mixing the below-listed ingredients in proportions by weight as follows:

|                                  | Per cent |
|----------------------------------|----------|
| Crepe rubber                     | 30.2     |
| Bentonite                        | 30.2     |
| Woodpulp treated (dry basis)     | 15.1     |
| Sulfur                           | 15.1     |
| Diphenylguanidine                | 1.5      |
| Active organic ligneous compound | 0.5      |
| Water                            | 7.4 75   |

The active organic ligneous compound, which is insoluble in water and sulfuric acid, may be added either as a dry powder or as a liquid and is thoroughly mixed with the other constituents in order to obtain good distribution throughout the separator mass.

The separator mass is then formed or molded by a pressure operation, such as by passing it between suitable rolls, and then vulcanized with heat, preferably in a moist atmosphere. The formed product is then cut up into separators of the desired shape and size. The finished separator should contain sufficient voids or porosity so as to permit free passage of the electrolyte through the separator when it is assembled into the battery. The percentage of the voids will vary depending upon the constituents used in making the composition separators. However, it is desirable that the voids constitute at least 50% of the separator volume.

Composition separators obtained from the foregoing example were made up into standard type lead-acid storage batteries. These batteries were then subjected to a standard discharge test in comparison with other batteries made up with composition separators fabricated from identical ingredients but not containing the active organic ligneous compounds. The technique on the tests was as follows:

The batteries undergoing automatic life tests were subjected to a discharge of 300 amperes at 0° F. and a cut-out of one volt per cell or 3 volts for the entire battery. When the battery was completely discharged, it was fully charged and again discharged under the same test conditions, the discharge and charge being considered as one cycle. As the cycles of discharge and charge follow one upon the other, the duration of time of the discharge portion of the cycle becomes shorter, so that after any given number of cycles that battery whose discharge output is greater than another battery is said to have a better low temperature capacity characteristic.

Under these conditions the results obtained in testing the batteries prepared with the separators obtained according to the aforesaid example and those obtained with batteries containing untreated separators were as follows:

|                        | No. of cycles | Duration of discharge portion of cycle-seconds |           |
|------------------------|---------------|------------------------------------------------|-----------|
|                        |               | Treated                                        | Untreated |
| Composition separators | 253           | 200                                            | 80        |

The improved result of our invention is most pronounced at the period when it is most needed, namely, after numerous cycles of discharge and charge and particularly effective under the most severe operating conditions, viz., cold weather. Furthermore, the improved result is not dependent upon nor associated with the presence of an organic expander in the negative plate. The improvement of the present invention is obtained regardless of whether the negative plate of the battery contains an organic expander or not. Where expanders are used in the negative plates in conjunction with the present invention, it appears that the effect of the improved separator makes itself felt most prominently about the time the effect of the organic expanders of the negative plate begins to be dissipated.

When the novel separators of the present in-

vention are incorporated into storage batteries of the lead-acid type, batteries are obtained which possess greater discharge output capacity and longer life, especially at low temperatures, which, over a 300-350 cycle life test period, is seldom less than 40 per cent greater than a similar battery containing the separators of the prior art and in many cases is as much as 100 or more per cent greater.

By virtue of the improved results above set forth, it is easily possible to distinguish between my improved composition separators and those of the prior art. However, a simpler and quicker test for identifying my improved separators from those of the prior art is to cut up the respective separators and treat the pieces with a 2-3% caustic soda solution. The extracted matter dissolved from my improved composition separator will, because of the presence of the active organic ligneous compound, impart to the caustic soda solution a considerably intensified color which will be lacking in the case of ordinary separators.

Having thus described my invention, I claim the following as new and useful:

1. Method of manufacturing an improved composition storage battery separator composed essentially of porous rubber which comprises intimately mixing a small amount of an active organic ligneous compound with the primary constituents from which the separator is fabricated and thereafter fabricating the separator.

2. Method of manufacturing an improved composition storage battery separator composed essentially of porous rubber which comprises intimately and uniformly mixing a small amount of an active organic ligneous compound in the form of a dry powder with the primary constituents from which the separator is fabricated and thereafter fabricating the separator.

3. Method of manufacturing an improved composition separator composed essentially of porous rubber which comprises intimately and uniformly mixing a small amount of an active

organic ligneous compound in the form of a liquid with the primary constituents from which the separator is fabricated and thereafter fabricating the separator.

5. Method of manufacturing an improved composition separator composed essentially of porous rubber which comprises intimately and uniformly mixing with the primary constituents from which the separator is fabricated an amount of an active organic ligneous compound between about 0.01 per cent and about 5.0 per cent by weight and thereafter fabricating the separator.

10 15 20 25 30 35 40

6. Method of manufacturing an improved composition separator composed essentially of porous rubber which comprises intimately and uniformly mixing with the primary constituents from which the separator is fabricated an amount of an active organic ligneous compound between about 0.25 and about 2.0 per cent by weight and thereafter fabricating the separator.

7. A composition storage battery separator composed essentially of porous rubber having incorporated therein a small amount of an active organic ligneous compound.

8. A composition storage battery separator composed essentially of porous rubber containing uniformly distributed throughout its pores and upon its surfaces a small amount of an active organic ligneous compound.

9. A composition storage battery separator composed essentially of porous rubber having as one of the ingredients thereof an active organic ligneous compound in an amount between about 0.01 per cent and about 5.0 per cent based on the weight of the separator.

10 15 20 25 30 35 40

10. A composition storage battery separator composed essentially of porous rubber having as one of the ingredients thereof an active organic ligneous compound in an amount between about 0.25 per cent and about 2.0 per cent based on the weight of the separator.

BRUNO H. SCHUBERT.